

# UNITED STATES PATENT OFFICE.

LOUIS J. CURTMAN, OF NEW YORK, N. Y.

## ERIQUET AND METHOD OF PRODUCING THE SAME.

1,173,779.

Specification of Letters Patent.

Patented Feb. 29, 1916.

No Drawing.

Application filed May 20, 1913. Serial No. 768,697.

*To all whom it may concern:*

Be it known that I, LOUIS J. CURTMAN, a citizen of the United States, residing at the city of New York, borough of Manhattan, in the county and State of New York, have invented certain new and useful Improvements in Briquets and Methods of Producing the Same, of which the following is a full, clear, and exact specification.

10 My invention relates to improvements in the production of briquets from pulverulent, or granulated material, and the same has for its object, more particularly to provide a briquet consisting essentially of fuel and a 15 binder so combined and treated as to form a body which shall be smokeless, odorless and water-proof, and which will burn without appreciable increase of ash.

Further said invention has for its object 20 to provide a briquet possessing such degree of hardness that it will not crumble or mat under storage conditions, and which will burn without disintegration or losing its form.

25 Further said invention has for its object to provide a method of producing briquets of the character hereinabove specified which is simple, effective and inexpensive, and which may be carried out by means of 30 apparatus usually employed in the briquetting of fuel and ores.

To the attainment of the aforesaid objects and ends my invention consists in the successive steps hereinafter described and in 35 the article or briquet, resulting in the carrying out of said steps.

For the purpose of illustration, I shall describe my invention as carried out in the production of briquet formed from anthracite coal. It will be understood however, 40 that the invention is not limited to use in connection with anthracite coal but is equally applicable to the briquetting of bituminous, culm and breeze, as well as mineral 45 ores.

In the production of briquetting from anthracite coal, the coal dust is preferably first passed through a grinder in order to reduce the coal and lumps therein to a uniform size, 50 and then discharged into a suitable receptacle and mixed with the required amount of binder.

As the binding agent, I preferably employ a composition produced by intimately 55 mixing about ninety (90) parts of crude molasses, technically known a black strap,

about nine (9) parts of highly concentrated and neutralized syrup of sulfite pitch, obtained by neutralizing with lime the waste sulfite liquor produced in the manufacture 60 of paper pulp, and about one (1) part of water gas tar. The binder and coal dust are mixed together cold, and when thoroughly mixed are molded in a briquet press. Upon leaving the press, the briquets 65 are not hard nor water-proof, and if placed in a fire at this stage of the process they would be far from smokeless.

To render the briquets hard, water-proof, and smokeless, I then subject the molded 70 mass to a baking action for about one hour. The baking of the briquets is performed in an oven preferably formed with a plurality of compartments in which the temperature is gradually or successively increased from 75 about 250 to 500 degrees Fahr. By this means the water is practically all volatilized at the relatively low temperature, and at the same time the molasses is concentrated and caused to spread more thoroughly 80 throughout the entire mass and coat each of the particles of coal dust. At the higher temperatures the concentrated molasses undergoes a chemical change, the net result of 85 which is the production of a coke-like mass which knits the coal particles into a hard, water-proof body, which will thereafter burn without smoke or odor.

I have found that a binder composed of 90 crude molasses when combined with concentrated and neutralized syrup of sulfite pitch, and water gas tar, is particularly desirable for, and may be used with advantage and economy in binding ores and inferior 95 grades of fuels.

It is to be noted that the specific proportions of the several elements of the binder may be varied within reasonable limits in order to adapt the same to different kinds of ores or fuels, and that the amount of 100 binder required in any instance to produce satisfactory briquets, will of course depend upon the quantity of water or liquid present in the material to be bonded.

Having thus described my invention, what 105 I claim and desire to secure by Letters Patent is:

1. A briquet consisting of granulated fuel mixed with a binder containing molasses and water gas tar, molded to shape and 110 baked, substantially as specified.

2. A briquet consisting of granulated coal

combined with a binder composed of molasses, concentrated and neutralized syrup of sulfite pitch, and water gas tar, molded to shape, and baked, substantially as specified.

3. A briquet consisting of granulated coal combined with a binder composed of crude molasses concentrated and neutralized syrup of sulfite pitch, and water gas tar, molded to shape, and baked substantially as specified.

4. A briquet consisting of granulated coal combined with a binder composed of crude molasses (about 90 parts), concentrated and neutralized syrup of sulfite pitch (about 9 parts), and water gas tar (about 1 part) molded to shape, and baked, substantially as specified.

5. The method of forming briquets consisting in combining granulated material with a binder composed essentially of a carbo-hydrate, and water gas tar, molding the same to shape, and then baking said molded mass, substantially as specified.

6. The method of forming briquets which consists in combining granulated material with a binder composed essentially of molasses, and water gas tar, molding the same

to shape, and then baking said molded mass, substantially as specified.

7. The method of forming briquets which consists in combining granulated coal with a binder composed essentially of molasses, and water gas tar, molding the same to shape, and then baking said molded mass for about one hour at a gradually increasing temperature, up to 500 degrees Fahr., substantially as specified.

8. The method of forming briquets which consists in combining granulated fuel with a binder containing molasses and water gas tar, molding the same to shape, subjecting the molded mass to a temperature sufficient to volatilize water and to cause the molasses to spread throughout the mass, and then subjecting the molded mass to a higher temperature to convert the binder into a coke-like mass, substantially as specified.

Signed at the city of New York, in the county and State of New York, this 14th day of May, one thousand nine hundred and thirteen.

LOUIS J. CURTMAN.

Witnesses:

CONRAD A. DIETERICH,  
JOSEPH G. QUINN, JR.